

No. 728,778.

PATENTED MAY 19, 1903.

H. SPECKETER.

PRODUCTION OF CHROMIUM COMPOUNDS AND ALKALIES.

APPLICATION FILED JULY 1, 1901.

NO MODEL.



Fig. 1.



Fig. 2.

Witnesses

Jeffinkel

John Gillman, Jr.

By

Peter Freeman

Attorneys

Inventor  
Heinrich Specketer

## UNITED STATES PATENT OFFICE.

HEINRICH SPECKETER, OF GRIESHEIM-ON-THE-MAIN, GERMANY, ASSIGNEE  
TO CHEMISCHE FABRIK GRIESHEIM ELECTRON, OF FRANKFORT-ON-THE-  
MAIN, GERMANY, A FIRM.

## PRODUCTION OF CHROMIUM COMPOUNDS AND ALKALIES.

SPECIFICATION forming part of Letters Patent No. 728,778, dated May 19, 1903.

Application filed July 1, 1901. Serial No. 66,747. (No specimens.)

*To all whom it may concern:*

Be it known that I, HEINRICH SPECKETER, a subject of the Emperor of Germany, and a resident of 1 Bahnstrasse, Griesheim-on-the-  
5 Main, near Frankfort-on-the-Main, Germany, have invented certain new and useful Improvements in the Production of Chromium Compounds and Alkalies, of which the following is a specification.

10 The principal object of this invention is to provide a process for economically and on a commercial scale producing chromium compounds and alkalies. The said process consists, essentially, in subjecting to electrolysis  
15 the solution of any alkali-metal salt or of mixture of alkali-metal salts and using an anode of chromium or an alloy thereof or by using salts of chromium as an electrolyte with an insoluble anode, the anode electrolyte being separated from the cathode electrolyte by a diaphragm or other equivalent means preventing the said liquid becoming mixed, while hydroxids or carbonates are added to the electrolyte for the purpose of  
20 precipitating the alkali-metal salt with the chromium and neutralizing the free acid which is formed along with the chromic acid.

In the accompanying drawings there is represented a conventional form of battery which  
25 may be used in carrying out the process.

In the drawings, Figure 1 is a vertical section, and Fig. 2 is a horizontal section.

*a* represents the anode, *b* the cathode, and *c d* the diaphragms.

30 This invention can be carried out as follows: The electrolyte consists, for instance, of a solution of sodium sulfate. The anode is of ferrochromium, such as is obtained in the reduction of chrome-iron by carbon. The anode is separated from the cathode by a diaphragm. Calcium carbonate or caustic lime is added to the anode electrolyte. When an electric current is passed through the electrolyte, the following reactions take place:  
35 A soda-lye is produced in the cathode-compartment in accordance with the following equation:



40 In the anode-compartment free chromic

acid, free sulfuric acid, and ferric sulfate are formed, but undergo the following transformations in the electrolyte:

- (2.)  $2\text{FeCr} + 9\text{SO}_4 = \text{Fe}_2(\text{SO}_4)_3 + 2\text{Cr}(\text{SO}_4)_3$  55  
 (3.)  $\text{Cr}(\text{SO}_4)_3 + 4\text{H}_2\text{O} = \text{H}_2\text{CrO}_4 + 3\text{H}_2\text{SO}_4$ .  
 (4.)  $\text{H}_2\text{CrO}_4 + \text{H}_2\text{SO}_4 + 2\text{Ca}(\text{OH})_2 = \text{CaCrO}_4 + \text{CaSO}_4 + 2\text{H}_2\text{O}$ .  
 (5.)  $\text{Fe}_2(\text{SO}_4)_3 + 3\text{Ca}(\text{OH})_2 = \text{Fe}_2(\text{OH})_6 + 3\text{CaSO}_4$ . 60  
 (6.)  $\text{CaCrO}_4 + \text{Na}_2\text{SO}_4 = \text{Na}_2\text{CrO}_4 + \text{CaSO}_4$ .

The impurities pass into the precipitate and are separated by filtration, while the sodium chromate remains in the solution, which is evaporated to dryness or transformed by means of sulfuric acid into sodium bichromate.

Example: In an electrolytic bath divided 70 into anode and cathode compartments by means of a diaphragm are suspended an anode of ferrochromium and a cathode of iron. Into the cathode-compartment is introduced a saturated solution of sodium sulfate, and 75 into the anode-compartment is introduced a solution containing twenty-five per cent. of sodium sulfate, to which is added a quantity of caustic lime sufficient to neutralize one hundred grams of chromic acid per liter and 80 the corresponding quantity of iron. The voltage of the electric current is from two and one-half to three volts, and the amperage is from one and one-half to two amperes per square decimeter. When the concentration 85 of the chromic acid reaches about one hundred grams per liter, the solution is emptied, the iron hydroxid and gypsum separated by filtration, and the solution evaporated to crystallize the sodium chromate. The cathode-lye is likewise evaporated when its concentration amounts to fifty or sixty grams of soda-lye per liter, and the precipitated sodium sulfate can be used again in the process. 90

It is known that chromium and chromium alloys used as anode in a solution of alkali-metal salts pass into the solution as chromic acid. It is also known that the electrolysis of alkali-metal salts produces hydroxid at the cathode. If this process were carried out 100

without the use of a diaphragm or other device preventing the intermingling of the anode and cathode electrolytes, the process would be unprofitable. It is, however, rendered profitable by combining both the anode and cathode process in the hereinbefore-described manner and obtaining from salts of low value, such as sodium chloride or sodium sulfate, a valuable soda-lye, as well as chromates, which final products have all a good marketable value.

The special feature of the present process consists, therefore, in the simultaneous and combined electrolysis of chromium compounds and alkali-metal salts, whereby a valuable alkali and chromic acid are simultaneously obtained. Such a combined extraction of alkali and chromic acid from initial products of low value is neither described in the special literature nor has it hitherto, as far as is known, ever been carried out.

It should be further remarked that two diaphragms may be used in the aforesaid process and the free acid neutralized with lime or the like in the space between these two diaphragms. The neutralization of the anode-lye and the precipitation of the iron are then effected in another vessel.

Instead of using chromium or ferrochromium directly as anode it may be dissolved in sulfuric acid or bisulfate, and the process for obtaining the chromic acid and alkali is then as follows: As anode electrolyte a solution of chromium sulfate or of chromic-iron sulfate is used, which may be either neutral or acid. The cathode electrolyte consists of a solution of sodium sulfate. The anode and cathode electrolytes are separated from each other by a double diaphragm. In the intermediate space between the two diaphragms is also sodium sulfate, to which, for instance, lime or calcium carbonate is added. The cathode is of iron and the anode of lead. When the chromium sulfate is oxidized to chromic acid, which may be seen from the color, the solution is raised to the ebullition-

point—120° to 130° centigrade. The iron sulfate crystallizes out and is separated by filtration. To separate the chromic acid, the filtrate is boiled to a temperature of about 50° from 150° to 160° centigrade. The chromic acid is precipitated and separated by filtration. The filtrate contains still small quantities of chromic acid and of unoxidized chromium sulfate in the form of chromium sulfite and can be used again to dissolve ferrochromium. It is also possible by evaporating the original solution to from 150° to 160° centigrade to precipitate both the iron sulfate and the chromic acid and extract the chromic acid from the mixture by means of water or sulfuric acid. The ferric sulfate is washed out with water or sulfuric acid in order to remove the chromic acid included therein.

Having now particularly described and ascertained the nature of the said invention and in what manner the same is to be performed, I declare that what I claim is—

1. The process, substantially as herein described, of producing chromium compounds and alkalies, which consists in electrolyzing solutions of the salts of the alkalies with an anode containing chromium, while preventing the intermingling of the anode and cathode electrolytes and adding to the anode electrolyte a neutralizing agent.

2. The process, substantially as herein described, of producing chromium compounds and alkalies, which consists in electrolyzing solutions of the salts of the alkalies with an anode containing chromium, while preventing the intermingling of the anode and cathode electrodes and adding to the anode electrode a hydroxid.

In testimony whereof I have signed my name to this specification in the presence of two subscribing witnesses.

HEINRICH SPECKETER.

Witnesses:

FRANZ HASSSLACHER,  
MICHAEL VOLK.